

## 1

3,294,501

**CORROSION INHIBITORS FOR GASOLINES**  
 Fred K. Kawahara, Park Forest, Ill., assignor to Standard  
 Oil Company, Chicago, Ill., a corporation of Indiana  
 No Drawing. Filed Nov. 13, 1964, Ser. No. 411,146  
 1 Claim. (Cl. 44—71)

This is a continuation-in-part of U.S. patent application Ser. No. 234,557, now abandoned.

This invention relates to corrosion inhibitors for gasolines. More particularly it relates to the use of certain corrosion inhibitors for gasolines which contain tetra-alkyl lead and a benzoic-acid or a hexahydrobenzoic-acid-type lead appreciator.

For the most part, motor gasolines that are marketed in this country contain tetra-alkyl lead compounds such as tetramethyl or tetraethyl lead to upgrade their octane ratings. Recently, it has been found that certain organic compounds possess the unusual feature of enhancing the effectiveness of tetra-alkyl lead compounds. Two such compounds are benzoic acid and hexahydrobenzoic acid (i.e., cyclohexane carboxylic acid). This phenomenon of enhancing the effectiveness of tetra-alkyl lead compounds is termed "lead appreciation" and is currently receiving scientific as well as commercial attention.

Both benzoic acid and hexahydrobenzoic acid are very corrosive with respect to several metals, particularly when in contact with moisture. Gasolines containing either of these compounds are particularly corrosive toward zinc or zinc alloys. Both zinc and zinc alloys are used extensively in fuel pumps, carburetors and other die-cast parts of automotive and aviation engines.

It has now been discovered pursuant to the invention that the corrosiveness toward zinc and zinc alloys of gasolines containing either benzoic acid or hexahydrobenzoic acid as a lead appreciator may be substantially inhibited by incorporating into the gasoline a small amount of one or more of the following additives:

Picric acid  
 3,5-dinitrosalicylic acid  
 5-nitrosalicylic acid  
 1-hydroxy-2-naphthoic acid  
 3-hydroxy-2-naphthoic acid  
 2,4,5-trihydroxy butyrophenone  
 5,5'-methylene disalicylic acid  
 2,4-dinitrophenol

It has been found that the effectiveness of the foregoing inhibitors may be considerably enhanced, in certain cases, by utilizing a combination of inhibitors, as will be shown presently.

An additional discovery associated with the present invention is that the effectiveness of the foregoing inhibitors may be enhanced even further by adding to the inhibited gasoline a small amount of trihydroxy decanophenone, which is, by itself an ineffective corrosion inhibitor. It has been demonstrated also that many compounds which may be suggested by the prior art as inhibiting ferrous-metal corrosion and which are close analogs of the inventive additives fail to exhibit any substantial degree of inhibition of corrosion of zinc in the presence of benzoic acid or hexahydrobenzoic acid. This is clearly shown

## 2

by the results from tests made with such compounds as 2,4-dihydroxy benzoic acid, p-hydroxy benzoic acid, salicylic acid, beta-naphthoic acid, 2-hydroxy stearic acid, dl-mandelic acid and citrimic acid.

- 5 The various tests employed in this series of experiments, as well as those reported later, involved the following procedure. For each test, 100 ml. of leaded gasoline were poured into a tall-form bottle. In some of these tests, the leaded gasoline contained no other substances.  
 10 In others, the leaded gasoline contained 0.2% hexahydrobenzoic acid; and still in others, the leaded gasoline contained both hexahydrobenzoic acid and an anti-corrosion agent.

A weighted strip of metal was then immersed in each 15 gasoline sample. After a particular strip had been immersed for 30 minutes, 10 ml. of water were added and the bottle was rolled for one minute. After three days of immersion, each metal strip was removed, scrubbed, and washed to remove corrosion products and reweighed. The loss in weight was taken as a measure of effectiveness of the particular corrosion inhibitor. The results of this series of tests, which used strips of zinc metal and anti-corrosion agents suggested by the prior art, are reported in Table I below:

25

TABLE I

| Test | Gasoline Composition                                               | Zinc Loss, Mg. |
|------|--------------------------------------------------------------------|----------------|
| 30   |                                                                    |                |
| 1    | Leaded gasoline                                                    | 0.5            |
| 2    | As in Test 1 plus 0.2% cyclohexane carboxylic acid                 | 34.1           |
| 3    | As in Test 2 plus 2,4-dihydroxybenzoic acid (30 PTB <sup>1</sup> ) | 32.9           |
| 4    | As in Test 2 plus p-hydroxybenzoic acid (30 PTB <sup>1</sup> )     | 33.5           |
| 5    | As in Test 2 plus alicyclic acid (30 PTB <sup>1</sup> )            | 28.2           |
| 6    | Leaded gasoline                                                    | 2.9            |
| 7    | As in Test 6 plus 0.2% cyclohexane carboxylic acid                 | 30.8           |
| 8    | As in Test 7 plus 2-hydroxy stearic acid (30 PTB <sup>1</sup> )    | 30.4           |
| 9    | As in Test 7 plus dl-mandelic acid (30 PTB <sup>1</sup> )          | 31.9           |
| 10   | Leaded gasoline                                                    | 0.5            |
| 11   | As in Test 10 plus 0.2% cyclohexane carboxylic acid                | 31.3           |
| 12   | As in Test 11 plus citrimic acid (30 PTB <sup>1</sup> )            | 25.8           |

40

<sup>1</sup> Concentration of additive in pounds per thousand barrels of gasoline.

The results of Tests 2, 7 and 11 demonstrate that hexahydrobenzoic acid, i.e., cyclohexane carboxylic acid, is very corrosive toward zinc. The results of Tests 3, 4 and 5 indicate that 2,4-dihydroxybenzoic acid, p-hydroxybenzoic acid and salicylic acid, individually, did not appreciably reduce the corrosive action of the cyclohexane carboxylic acid on the zinc. Furthermore, the results of Tests 8, 9 and 12 indicate that 2-hydroxy stearic acid, dl-mandelic acid and citrimic acid, individually, did not reduce the corrosiveness of the cyclohexane carboxylic acid toward zinc.

These results establish that anti-corrosion inhibitors of the six types suggested by the prior art do not inhibit the corrosion of zinc resulting from the presence of cyclohexane carboxylic acid (hexahydrobenzoic acid).

The quantities of the inventive additives that are incorporated into gasolines for internal combustion engines are not crucial. These quantities depend upon the 55 amount of the benzoic acid or hexahydrobenzoic acid (cyclohexane carboxylic acid) that is present, the service conditions of storage and use, the nature of the inhibitor, and other similar factors. It has been found that excellent corrosion inhibition is obtained at additive concentra-

tions of as little as 30 pounds of additive per thousand barrels of gasoline (42 gallons per barrel), although this amount may be increased or decreased as a matter of preference. Quantities as little as 0.5 pound per thousand barrels of gasoline, or even less, are effective, while quantities of as much as 100 pounds per thousand barrels, or more, may be used in a particularly serious situation.

The other constituents of the gasoline will depend upon the manufacturers' specifications and the consumers' requirements. Ordinarily, the gasoline is predominantly a hydrocarbon, having paraffin, naphthene, olefin and aromatic constituents. It contains a tetra-alkyl lead at a concentration ordinarily within the range of 0.5 to about 6 cubic centimeters per gallon, depending upon market requirements. It also may contain either benzoic acid or hexahydrobenzoic acid, advantageously in the free-acid form, although derivatives such as the methyl or other gasoline-soluble esters may be used. The amount of the benzoic acid or hexahydrobenzoic acid may range from as little as 0.005 weight percent to about 1.0 weight percent. As was noted above, this quantity is not critical and may be greater or smaller than the foregoing range for as much as an order of magnitude, if this is required.

The inventive additives were evaluated in a number of tests employing the simple laboratory tests discussed above. In some of these tests, the corrosive action of hexahydrobenzoic acid, as inhibited by selected compounds, was determined with iron and copper strips, as well as zinc strips. In each case the metal strips were of uniform size, about  $2\frac{1}{2}$  inches long by  $\frac{1}{2}$  inch wide. Each zinc strip weighed approximately 1.5 gr.; each iron strip weighed about 2.4 gr.; and each copper strip, about 3.7 gr.

In the first series of tests, benzoic acid was used as the lead appreciator and zinc strips were employed. The results from the tests of this series are presented in Table II.

TABLE II

| Test | Gasoline Composition                                                     | Zinc Loss, Mg., After— |         |
|------|--------------------------------------------------------------------------|------------------------|---------|
|      |                                                                          | 3 Days                 | 5 Days  |
| 13   | Leaded gasoline                                                          | 0.5                    |         |
| 14   | Leaded gasoline and 0.2% benzoic acid                                    | 29.8-35.2              | 39.3    |
| 15   | As in Test 14 plus 2,4,5-trihydroxy butyrophenone (30 PTB <sup>1</sup> ) | 3.7-4.0                | 4.5-6.0 |

<sup>1</sup> Concentration of additive in pounds per thousand barrels of gasoline. The results of Test 14 show the corrosive action of the benzoic acid toward zinc. The results from Test 15 show the inhibition of such corrosion by the use of 2,4,5-trihydroxy butyrophenone.

In the second series of tests, hexahydrobenzoic acid (cyclohexane carboxylic acid) was used as the lead appreciator. A number of organic compounds was used to inhibit the corrosive effect of the lead appreciator on zinc. In addition, various combinations of these inhibitors were employed. In general, the concentration of an inhibitor, when used alone, was 30 pounds of the inhibitor per 1000 barrels of the gasoline. In the case of the use of multiple inhibitors, the total quantity of the inhibitors did not exceed 30 pounds per 1000 barrels. Equal portions of the inhibitors were employed; for example, in Test 29 corrosive inhibition of the zinc was brought about by the use of 15 pounds of 3-hydroxy-2-naphthoic acid per 1000 barrels of gasoline and 15 pounds of 2,3,4-trihydroxy decanophenone per 1000 barrels of gasoline, while in Test 36 corrosion inhibition resulted from the use of 10 pounds of picric acid per 1000 barrels of gasoline, 10 pounds of 5-nitrosalicylic acid per 1000 barrels of gasoline and 10 pounds of 3,5-dinitrosalicylic acid per 1000 barrels of gasoline. The results of the tests made in this series are presented in Tables III and IV.

TABLE III

| Test | Gasoline Composition                                                        | Concentration, PTB <sup>1</sup> | Zinc Loss After Specified No. of Days, Mg. |         |           |      |      |      |     |
|------|-----------------------------------------------------------------------------|---------------------------------|--------------------------------------------|---------|-----------|------|------|------|-----|
|      |                                                                             |                                 | 3                                          | 4       | 6         | 14   | 42   | 70   | 105 |
| 16   | Leaded gasoline                                                             | 0.5                             |                                            |         |           |      |      |      |     |
| 17   | Leaded gasoline and 0.2% hexahydrobenzoic acid                              | 29.6-34.1                       | 0.3-1.4                                    | 0.5-2.9 | 2.8       | 0.6  | 0.3  | 0.2  |     |
| 18   | As in Test 17 plus picric acid                                              | 30                              | 27.4-33.0                                  | 30.8    | 31.1-31.8 | 34.2 | 42.3 | 42.1 |     |
| 19   | As in Test 17 plus 3,5-dinitrosalicylic acid                                | 30                              | 2.1/6.8                                    | 1.5     | 11.1      |      |      |      |     |
| 20   | As in Test 17 plus 5-nitrosalicylic acid                                    | 30                              | 6.8                                        |         | 16.3      |      |      |      |     |
| 21   | As in Test 17 plus 1-hydroxy-2-naphthoic acid                               | 30                              | 2.9                                        |         |           |      |      |      |     |
| 22   | As in Test 17 plus 3-hydroxy-2-naphthoic acid                               | 30                              | 2.2                                        |         | 5.9       | 21.7 |      |      |     |
| 23   | do                                                                          | 15                              |                                            |         | 21.1      |      |      |      |     |
| 24   | As in Test 17 plus 5,5'-methylene disalicylic acid                          | 30                              | 7.1                                        |         |           |      |      |      |     |
| 25   | As in Test 17 plus 4-ethoxy-2-hydroxybenzoic acid                           | 30                              | 9.2                                        |         |           |      |      |      |     |
| 26   | As in Test 17 plus 2,4-dinitrophenol                                        | 30                              |                                            | 5.1     |           |      |      |      |     |
| 27   | As in Test 17 plus 3,5-dinitrosalicylic acid and 3-hydroxy-2-naphthoic acid | { 15                            |                                            |         |           | 2.2  | 2.3  |      |     |

<sup>1</sup> Concentration of additives in pounds per thousand barrels of gasoline.

TABLE IV

| Test | Gasoline Composition                                                                             | Concentration, PTB <sup>1</sup> | Zinc Loss After Specified No. of Days, Mg. |      |      |     |      |
|------|--------------------------------------------------------------------------------------------------|---------------------------------|--------------------------------------------|------|------|-----|------|
|      |                                                                                                  |                                 | 4                                          | 14   | 42   | 70  | 105  |
| 28   | As in Test 17 plus 2,3,4-trihydroxy decanophenone                                                | 30                              | 23.0                                       |      |      |     |      |
| 29   | As in Test 17 plus 3-hydroxy-2-naphthoic acid and 2,3,4-trihydroxy decanophenone                 | { 15                            |                                            | 0.7  | 5.2  | 3.3 | 4.7  |
| 30   | As in Test 17 plus 3-hydroxy-2-naphthoic acid and 2,3,4-trihydroxy decanophenone                 | { 15                            |                                            | 1.1  | 19.0 |     |      |
| 31   | As in Test 17 plus picric acid and 3-hydroxy-2-naphthoic acid                                    | { 15                            |                                            | 1.9  | 21.4 | 3.6 | 32.1 |
| 32   | As in Test 17 plus picric acid and 3-hydroxy-2-naphthoic acid                                    | { 15                            |                                            | 24.2 | 33.7 |     |      |
| 33   | As in Test 17 plus 3,5-dinitrosalicylic acid and 3-hydroxy-2-naphthoic acid                      | { 15                            |                                            | 2.2  | 2.3  |     |      |
| 34   | As in Test 17 plus 3,4-dinitrosalicylic acid and 3-hydroxy-2-naphthoic acid                      | { 15                            |                                            | 4.8  | 12.7 |     |      |
| 35   | As in Test 17 plus picric acid and 5-nitrosalicylic acid                                         | { 15                            |                                            |      |      | 4.6 | 4.0  |
| 36   | As in Test 17 plus picric acid and 5-nitrosalicylic acid and 3,5-dinitrosalicylic acid           | { 10                            |                                            |      |      | 3.7 | 4.4  |
| 37   | As in Test 17 plus picric acid and 3-hydroxy-2-naphthoic acid and 2,3,4-trihydroxy decanophenone | { 10                            |                                            |      |      | 0.9 | 0.8  |

<sup>1</sup> Concentration of additive in pounds per thousand barrels of gasoline.

The corrosive nature of hexahydrobenzoic acid toward zinc is clearly shown by Test 17. Examination of the re-

to inhibit the corrosive effect of hexahydrobenzoic acid on zinc. The results of these tests are shown in Table VI.

TABLE VI

| Test | Gasoline Composition                                                                             | Immer-<br>sion<br>Days | Zinc Loss, Mg. |              |
|------|--------------------------------------------------------------------------------------------------|------------------------|----------------|--------------|
|      |                                                                                                  |                        | Fresh<br>Water | Sea<br>Water |
| 48   | Leaded gasoline                                                                                  | 33                     | 0.4            | 2.2          |
| 49   | Leaded gasoline and 0.2% hexahydrobenzoic acid                                                   | 33                     | 28.4           | 32.0         |
| 50   | As in Test 49 plus picric acid and 3-hydroxy-2-naphthoic acid and 2,3,4-trihydroxy decanophenone | 33                     | 0.3            | 1.0          |
| 51   | Leaded gasoline                                                                                  | 70                     | 0.3            | 15.3         |
| 52   | Leaded gasoline and 0.2% hexahydrobenzoic acid                                                   | 70                     | 43.3           | 40.2         |
| 53   | As in Test 52 plus picric acid and 3-hydroxy-2-naphthoic acid and 2,3,4-trihydroxy decanophenone | 70                     | -----          | 1.8          |

sults from Tests 18-28 show the effectiveness of the various compounds in inhibiting the corrosion of zinc due to the presence of hexahydrobenzoic acid. Only the compound used in Test 28, 2,3,4-trihydroxy decanophenone, does not greatly reduce the corrosion. However, the use of 2,3,4-trihydroxy decanophenone in conjunction with another additive improves the corrosion inhibition due to the use of the other additive. Compare the results from Test 22 with those from Test 29. Furthermore, combinations of the various compounds seem to inhibit the corrosive effect toward zinc, at least when the combinations are used in a concentration of 30 pounds of inhibitors per 1000 barrels of gasoline. For example, in Test 31, the combination of picric acid and 3-hydroxy-2-naphthoic acid in a combined concentration of 30 pounds per 1000 barrels of gasoline inhibits the corrosive action at least after 14 days of immersion. However, when the total concentration was halved, as shown in Test 32, substantial corrosion had occurred after the same period of time.

The results of the tests made with the iron and copper strips are presented in Table V.

TABLE V

| Test | Gasoline Composition                                                             | Concen-<br>tration,<br>PTB <sup>1</sup> | Metal Loss After Specified No.<br>of Days, Mg. |       |       |        |       |       |
|------|----------------------------------------------------------------------------------|-----------------------------------------|------------------------------------------------|-------|-------|--------|-------|-------|
|      |                                                                                  |                                         | Iron                                           |       |       | Copper |       |       |
|      |                                                                                  |                                         | 4                                              | 14    | 42    | 4      | 14    | 42    |
| 38   | Leaded gasoline                                                                  | -----                                   | 0.8                                            | 3.7   | 2.8   | 0.0    | 0.3   | 0.5   |
| 39   | Leaded gasoline and 0.2% hexahydrobenzoic acid                                   | -----                                   | 6.6                                            | 5.9   | 5.4   | 3.8    | 7.1   | 9.4   |
| 40   | As in Test 39 plus picric acid                                                   | 30                                      | 1.3                                            | ----- | 4.6   | -----  | ----- | ----- |
| 41   | As in Test 39 plus 2,3,4-trihydroxy decanophenone                                | 30                                      | 0.9                                            | ----- | 1.3   | -----  | ----- | ----- |
| 42   | As in Test 39 plus 3-hydroxy-2-naphthoic acid and 2,3,4-trihydroxy decanophenone | { 15<br>15 }                            | 3.1                                            | 2.8   | ----- | 1.8    | 2.7   | ----- |
| 43   | As in Test 39 plus 3-hydroxy-2-naphthoic acid and 2,3,4-trihydroxy decanophenone | { 7.5<br>7.5 }                          | 3.4                                            | 3.0   | ----- | 4.1    | 6.3   | ----- |
| 44   | As in Test 39 plus picric acid and 3-hydroxy-2-naphthoic acid                    | { 15<br>15 }                            | 1.5                                            | 0.6   | ----- | 0.9    | 1.1   | ----- |
| 45   | As in Test 39 plus picric acid and 3-hydroxy-2-naphthoic acid                    | { 7.5<br>7.5 }                          | 1.2                                            | 0.4   | ----- | 1.8    | 1.1   | ----- |
| 46   | As in Test 39 plus 3,5-dinitrosalicylic acid and 3-hydroxy-2-naphthoic acid      | { 15<br>15 }                            | 1.3                                            | 0.6   | ----- | 1.1    | 1.2   | ----- |
| 47   | As in Test 39 plus 3,5-dinitrosalicylic acid and 3-hydroxy-2-naphthoic acid      | { 7.5<br>7.5 }                          | 4.2                                            | 4.3   | ----- | 1.5    | 1.4   | ----- |

<sup>1</sup> Concentration of additive in pounds per thousand barrels of gasoline.

These results demonstrate that the use of the inventive compounds will not deteriorously affect these metals. Hence, they can be used safely to inhibit the corrosive nature of the benzoic acid or hexahydrobenzoic acid toward zinc without seriously affecting the iron and copper in the system.

In another series of tests, sea water, as well as fresh water, was used. The sea water was a synthetic preparation made according to the specification of ASTM Preparation D-665. The zinc strips were immersed in the various solutions for either 33 or 70 days. A combination of picric acid, 3-hydroxy-2-naphthoic acid, and 2,3,4-trihydroxy decanophenone, each in a concentration of 10 pounds per 1000 barrels of gasoline, was employed

and a second additive, said first additive being employed in conjunction with said second additive, said first additive comprising at least one member of the group consisting of:

Picric acid  
3,5-dinitrosalicylic acid  
5-nitrosalicylic acid  
1-hydroxy-2-naphthoic acid  
3-hydroxy-2-naphthoic acid  
2,4,5-trihydroxy butyrophenone  
5,5'-methylene disalicylic acid  
2,4-dinitrophenol,

said second additive being 2,3,4-trihydroxy decanophenone, the amount of said first additive being effective to

provide inhibition of the corrosiveness of gasoline containing water with respect to zinc, and the amount of said second additive being effective to improve said inhibition which results from the use of said first additive.

**References Cited by the Examiner**

**UNITED STATES PATENTS**

|           |         |                  |        |
|-----------|---------|------------------|--------|
| 2,334,158 | 11/1943 | Von Fuchs et al. | 44—70  |
| 2,349,044 | 5/1944  | Jahn             | 106—14 |

|           |         |                |         |
|-----------|---------|----------------|---------|
| 2,366,074 | 12/1944 | Wasson et al.  | 252—57  |
| 2,717,196 | 9/1955  | Wachter et al. | 252—393 |
| 3,062,612 | 11/1962 | Boucher        | 252—393 |

**FOREIGN PATENTS**

|         |        |            |
|---------|--------|------------|
| 230,132 | 9/1960 | Australia. |
|---------|--------|------------|

**DANIEL E. WYMAN, Primary Examiner.**

**Y. H. SMITH, Assistant Examiner.**